# EUROPEAN PATENT APPLICATION

(11) **EP 4 628 610 A1**
(43) Date of publication of application: **08.10.2025**
(21) Application number: 23898427.2
(22) Date of filing: 20.10.2023
(51) Int. Cl.: C22C 21/00

(54) **ALUMINIUM-BASED ALLOY**

(30) Priority: 02.12.2022 RU 2022131428
(71) Applicant: Obshchestvo S Ogranichennoj Otvetstvennost'Yu "Institut Legkikh Materialov I Tekhnologij", Moscow 119049 (RU)
(72) Inventor: MANN, Viktor Khrist'yanovich, g. Krasnoyarsk, 660111 (RU); KROKHIN, Aleksandr Yur'evich, g. Krasnoyarsk, 660111 (RU); RYABOV, Dmitrij Konstantinovich, g. Krasnoyarsk, 660111 (RU); VAKHROMOV, Roman Olegovich, g. Krasnoyarsk, 660111 (RU); GRADOBOEV, Aleksandr Yur'evich, g. Krasnoyarsk, 660111 (RU); IVANOVA, Anna Olegovna, g. Krasnoyarsk, 660111 (RU); NIKITINA, Margarita Aleksandrovna, g. Krasnoyarsk, 660111 (RU)
(74) Representative: Atalay, Baris
(86) International application number: PCT/RU2023/050246
(87) International publication number: WO 2024/117936

(57) **Abstract**

The invention refers to the metallurgy, in particular to non-heat-treatable wrought aluminium alloys based on the aluminium-magnesium-scandium system used as materials for elements of structures including welded structures. The non-heat-treatable wrought aluminium-based alloy contains, % wt: magnesium 3.0-5.2, manganese 0.15-1.0, scandium 0.01-0.045, zirconium 0.03-0.14, silicon 0.025-0.18, titanium 0.01-0.05, optionally yttrium, additionally at least one element of the group including copper and zinc in quantity of 0.01-0.55, at least one element of the group including boron and carbon in quantity of 0.01-0.05, aluminium and inevitable impurities as balance. The alloy is characterised by high values of strength, corrosion resistance, percentage elongation in the annealed state, as well as high workability.

## Description

### Field of invention

The invention refers to the non-ferrous metallurgy, in particular to non-heat-treatable workable aluminium alloys based on the aluminium-magnesium-scandium system used as materials for elements of structures including welded structures, which are fabricated also using the shaping operation.

### Technical level

A non-heat-treatable workable aluminium alloy based on the aluminium-magnesium-scandium system, which is widely used at present, is AMg5 grade alloy (as per GOST 4784-2019) with the following composition, % wt:

| | |
|---|---|
| Magnesium | 4.8-5.8 |
| Manganese | 0.3-0.8 |
| Titanium | 0.02-0.1 |
| Beryllium | 0.0002-0.005 |
| Aluminium | Balance |

### Impurities:

| | |
|---|---|
| Iron | Up to 0.5 |
| Silicon | Up to 0.5 |
| Copper | Up to 0.1 |
| Zinc | Up to 0.2 |

The alloy is widely used in various industries, such as ship building, aerospace engineering, construction, and transport machine building. The alloy is weldable using all welding procedures and highly corrosion-resistant. The main disadvantage of this alloy is its unsatisfactory strength.

There is a known non-heat-treatable wrought alloy designed for application in cold-moulded products with irregular shape, such as vessels, tanks, cans, etc. including welded structures (WO 2018/187406A1, C22C3/00, B32B15/01 published on October 11th, 2018). The alloy is designed for products, such as home appliance parts, construction elements, and vehicle body parts, which can be anodised.

The alloy has the following composition, % wt:

| | |
|---|---|
| Silicon | 0-0.1 |
| Iron | 0-0.2 |
| Copper | 0-0.3 |
| Manganese | 0-0.5 |
| Magnesium | 2.0-5.0 |
| Chromium | 0-0.2 |
| Zinc | 0-0.2 |
| Titanium | 0-0.1 |
| Aluminium | Balance |

A disadvantage of this alloy is its insufficient strength due to low contents of elements readily-soluble in aluminium, which ensure solid-solution hardening, and low quantity of transition metal additives, which ensure hardening through formation of dispersoids.

There is a known aluminium alloy of the Al-Mg system (patent #RU 2726520, C22C21/06 published on July 14th, 2020). The alloy is designed for production of wrought semi-finished products in form of plates, sheets, stamped parts, extrusion profiles for aerospace applications.

This alloy has the following chemical composition, % wt:

| | |
|---|---|
| Magnesium | 5.0-6.0 |
| Scandium | 0.06-0.16 |
| Beryllium | 0.0002-0.005 |
| Manganese | 0.15-0.6 |
| Zirconium | 0.01-0.12 |
| Zinc | 0.1-0.6 |
| Iron | 0.02-0.15 |
| Silicon | 0.01-0.1 |

### At least two elements selected from the group:

| | |
|---|---|
| Erbium | 0.03-0.16 |
| Hafnium | 0.01-0.16 |
| Ytterbium | 0.03-0.16 |
| Aluminium | Balance |

The main disadvantage of this alloy is its unsatisfactory mouldability due to high doping with hardening elements, in particular magnesium, while additional doping with rare-earth elements and scandium enhances the cold deformation effect. In addition, scandium content in the selected range results in low cost effectiveness of this alloy application due to high scandium cost. The alloy also contains beryllium, which has adverse health effects.

There is a known aluminium alloy with a micrograin structure of the aluminium-magnesium system, which can be used for production with the method of superplastic moulding of semi-finished products and parts in various industries (RU 2772479C1, C22C21/06 published on May 20th, 2022).

The alloy has the following composition, % wt:

| | |
|---|---|
| Magnesium | 4.5-5.5 |
| Zinc | 0.1-1.0 |
| Cerium | 0.6-1.2 |
| Iron | 0.5-0.9 |
| Manganese | 0.1-0.7 |
| Chromium | 0.05-0.20 |
| Zirconium | 0.1-0.3 |
| Scandium | 0.05-0.30 |
| Aluminium | Balance |

### Impurities:

| | |
|---|---|
| Silicon | Up to 0.16 |
| Titanium | Up to 0.10 |
| Copper | Up to 0.01 |
| Other impurities | Up to 0.20 |

A disadvantage of this alloy is its insufficient percentage elongation due to large quantity of elements, which ensure hardening through formation of dispersoids and decrease its plastic properties.

There is a known weldable corrosion-resistant aluminium-magnesium alloy with high magnesium content, which contains the triple aluminium-scandium-zirconium phase as a major component (patent #RU 2226565, C22C21/06 published on August 21st, 1998). The alloy is designed for fabrication of parts via welding and applied for air transport vehicles, primarily for fabrication of aircraft body parts.

The alloy has the following composition, % wt:

| | |
|---|---|
| Magnesium | 5.0-6.0 |
| Zirconium | 0.05-0.15 |
| Manganese | 0.05-0.12 |
| Titanium | 0.01-0.20 |

Some elements comprising the group:

| | |
|---|---|
| Scandium, terbium, cerium, and other lanthanides | 0.05-0.5 |

At that, it contains at least:

| | |
|---|---|
| Scandium | 0.1-0.2 |
| Copper and/or zinc | 0.1-0.4 |
| Inevitable silicon | Up to 0.1% |

### impurities

The main disadvantage of this alloy is negative impact from hardening elements on cold sheet stamping, in particular, with magnesium. Contents of scandium and other lanthanides in the selected range result in low cost effectiveness of this alloy application due to their high cost, as well as limited availability of lanthanides for batch production of semi-finished products made of this alloy.

There is a known aluminium-based alloy, which can be used for fabrication of products operating in corrosive environments and exposed to high loads including higher and cryogenic temperatures (patent #RU 2735846, 10 C22C21/08 published on November 9th, 2020). The alloy structure comprises aluminium solid solution and secondary precipitates.

The alloy has the following composition, % wt:

| | |
|---|---|
| Magnesium | 4.0-5.5 |
| Manganese | 0.3-1.0 |
| Iron | 0.08-0.25 |
| Chromium | 0.08-0.18 |
| Zirconium | 0.06-0.16 |
| Titanium | 0.02-0.15 |
| Scandium | 0.01-0.28 |
| Silicon | 0.08-0.18 |
| Vanadium (optionally) | 0.01-0.06 |
| Aluminium and inevitable impurities | Balance |

A disadvantage of this alloy is its insufficient mouldability due to high structural contents of secondary precipitate phases with L1₂ lattice containing zirconium and scandium over 0.18% vol. Chromium content, which is also declared in this alloy, may result in formation of coarse intermetallic compounds with negative effects on its mouldability in the cold stamping process as well.

The closest equivalent to the offered alloy is a non-heat-treatable aluminium alloy of grade 5182 (EN 573-3) with the following composition, % wt:

| | |
|---|---|
| Manganese | 0.2-0.5 |
| Magnesium | 4.0-5.0 |
| Aluminium | Balance |

### Impurities:

| | |
|---|---|
| Iron | Up to 0.35 |
| Silicon | Up to 0.2 |
| Copper | Up to 0.15 |
| Zinc | Up to 0.25 |
| Chromium | Up to 0.1 |
| Titanium | Up to 0.1 |

This alloy is applied in various industries including manufacturing of automotive sheets used for fabrication of panels with the methods of cold sheet stamping and stretching. The alloy has high workability allowing production of parts with the required geometry using the moulding operation. However, the alloy has low strength properties in the annealed state, which does not ensure the sufficient weight efficiency of products made of it.

### Invention disclosure

The invention objective is development of a non-heat-treatable wrought aluminium-based alloy for manufacturing of parts and structures (including welded structures), where the moulding operation can be used.

The technical result is solution of the stated problem, increase of strength keeping workability, corrosion resistance, and percentage elongation.

The technical result is achieved by means of the offered non-heat-treatable wrought aluminium-based alloy, which contains magnesium, manganese, scandium, zirconium, silicon, titanium, yttrium optionally (i.e. this means the alternative alloy composition with yttrium and without it), additionally contains at least one element of the group including copper and zinc, and additionally contains at least one element of the group including boron and carbon, with the following ratio of components, % wt:

| | |
|---|---|
| Magnesium | 3.0-5.2 |
| Manganese | 0.15-1.0 |
| Scandium | 0.010-0.045 |
| Zirconium | 0.03-0.14 |
| Silicon | 0.025-0.180 |
| Titanium | 0.01-0.05 |
| Yttrium (optionally) | 0.005-0.02 |
| At least one element of the group including copper and zinc (in total or separately) | 0.01-0.55 |
| At least one element of the group including boron and carbon (in total or separately) | 0.0001-0.005 |
| Aluminium and inevitable impurities | Balance |

According to the other aspect, the claimed invention refers to a product made of the aluminium alloy, which is described above.

'In total or separately' indication means total content of two elements or content of a separate (only one) element, while the range of values is the same in both cases.

### Brief drawing description

Fig. 1 shows a result of the Erikson test in form of an extruded dimple before failure.

### Invention embodiment

The following information on alloying components was surprisingly discovered during experimental tests of various alloy compositions:
Magnesium should be added in quantity from 3.0% wt to 5.2% wt into alloys to ensure the required strength properties. Further increase of magnesium content may negatively affect the material plasticity, complicate the production process of rolled semi-finished products, and reduce their corrosion resistance. Lower magnesium content does not ensure the required strength properties of alloys.

Addition of manganese in quantity from 0.15% wt to 1.0% wt further increases the material strength through formation of dispersoids and also improves the material mouldability. This effect is associated with the fact that manganese ensures precipitation of iron-containing phases in finer and more compact shapes.

Joint doping with scandium in quantity from 0.01% wt to 0.045% wt and zirconium in quantity from 0.03% wt to 0.14% wt ensures higher strength properties through formation of nano-sized dispersoids upon process heating during production of semi-finished products. In addition, these elements have a modifying effect on both cast and deformed structures of the material. Lesser recrystallised grain size facilitates deformation through sliding of grain boundaries and consequently has a positive effect on the material mouldability.

Addition of silicon in quantity over 0.025% wt increases the alloy strength thanks to solid-solution hardening, which consequently allows reducing quantity of expensive Sc for achievement of the required strength. However, silicon content over 0.18% wt results in formation of Mg₂Si crystallisation phase reducing workability during hot rolling, which has a negative effect. Presence of Mg₂Si phase is highly undesirable due to its insolubility during homogenisation annealing.

Addition of titanium in quantity from 0.01% wt to 0.05% wt ensures fine-grained structures after deformation through formation of compounds with aluminium being crystallisation centres during casting.

Doping with yttrium in quantity from 0.005% wt to 0.02% wt further increases strength, as well as improves corrosion resistance and mouldability thanks to modification of particle shapes of iron-containing phases to more favourable shapes.

Doping with elements from the group of copper and zinc in quantity from 0.01% wt to 0.55% wt in total or separately ensures further solid-solution hardening of the material. In addition, the natural material ageing process further improves hardening by precipitates. Al₈Mg₅ β-phase precipitates in large quantity at boundaries of grains in alloys with high magnesium content, which makes these alloys more susceptible to intercrystalline corrosion. Zinc precipitates serve as sites for initiation of Al₈Mg₅ deposition. This promotes deposition of Al₈Mg₅ phase both at boundaries and inside grains thereby reducing tendency to intercrystalline corrosion. Due to the fact that copper can form S'-Al₂CuMg particles, which precipitate at boundaries of grains and result in reduction of corrosion resistance, its content in the alloy should be limited to 0.55% wt.

In order to modify ingot structures and provide homogeneous grains with the regulated size after deformation in semi-finished products made of this alloy, at least one element of the group including boron and carbon is added in quantity from 0.0001% wt to 0.005% wt. The added elements form compounds with each other and aluminium being crystallisation centres during casting, which ensure fine-grained structures in ingots.

The provided Si ≤ Zr + 2Sc ratio allows excluding precipitation of triple phases with silicon and scandium and/or zirconium, formation of which may result in reduction of the dispersion hardening effect.

The offered alloy is not additionally doped with chromium in order to exclude formation of coarse intermetallic compounds, which deteriorate stampability.

In order to reduce adverse health effects for the operating personnel during production of the alloy, beryllium is not added as distinct from alloys with similar applications.

### Invention embodiment examples

### Example 1

Slabs 120x400x1200 mm in size were cast with the semi-continuous casting method. Chemical composition of the slabs is given in Table 1.

After cutting of the head and bottom parts, the slabs were homogenised in the three-stage mode. First stage at temperature of 310-320°C for 2 h. Second stage at temperature of 380-390°C for 4 h. Third stage at temperature of 420-440°C for 4 h. Blanks 100x340x320 mm in size for rolling were cut from the slabs after homogenisation. Hot rolling of the flat blanks was performed at temperatures of 400-440°C to thickness of 6 mm. After that, their intermediate annealing was performed at temperature of 290-330°C followed by cold rolling to thickness of 1.0 mm. The rolled sheets were annealed at temperature of 280-320°C.

Some specimens were cut from the sheets for tests of mechanical properties during tensioning at room temperature, corrosion resistance, and workability with the Erikson extrusion method.

The tensile tests were performed on the flat specimens according to GOST 1497-84. The process tests with the Erikson sheet extrusion method were performed according to GOST 10510-80. The intercrystalline corrosion tests were performed on the specimens 10x20 mm in size according to GOST 9.021-74 in solution 1 for 24 h.

The mechanical, process, and corrosion test results are given in Table 2.

**Table 2**

| Alloy composition | Mechanical properties at 20°C | | | Dimple depth, Erikson extrusion, mm | Intercrystalline corrosion, mm |
|---|---|---|---|---|---|
| | Ultimate tensile strength, σ_{B}, MPa | Yield strength σ_{0.2}, MPa | Percentage elongation δ, % | | |
| 1 | 310 | 195 | 20.5 | 8.0 | No |
| 2 | 320 | 170 | 23.5 | 8.7 | No |
| 3 | 320 | 160 | 23.0 | 8.2 | No |
| 4 | 300 | 163 | 27.4 | 9.2 | No |
| 5 | 333 | 197 | 21.0 | 8.5 | No |
| A (sheet, annealing) | 255 | 110 | 18.0 | 7.8 | No |

As the comparison of mechanical properties of the sheets given in Table 2 shows, the offered alloy ensures higher strength properties versus the prototype, whilst keeping percentage elongation, mouldability, and corrosion resistance. The most significant advantage of the alloy is higher strength, which will allow reducing wall thickness of products made of it and thereby increasing weight efficiency of structures made of it. The kept percentage elongation and results of the Erikson extrusion tests guarantee high workability of the material during moulding. An example of an extruded dimple before failure in the developed alloy composition is given in Fig. 1.

### Example 2

Billets D=178 mm were cast under the industrial conditions with the semi-continuous casting method with compositions given in Table 3 using the following charge materials: at least grade A85 aluminium, zinc in ingots, grade Mg-90 magnesium in ingots, Cu80F master alloy, grade Kr-90 crystalline silicon, Al-5Ti-1B modifying bars, double master alloys (Al-Zr10%, Al-Y2%, Al-Sc2%).

The billets were homogenised in the two-stage mode. First stage at temperature of 350°C for 4 h. Second stage at temperature of 450°C for 6 h. Profiles #1 with wall thickness of 6 mm were extruded from the billets. The billets were heated to temperature of 440-460°C before extrusion. The extrusion speed for all alloy compositions including the prototype was 0.3 mm/s. The surface quality and geometry of all extruded profiles met the required parameters, which in turn indicated the comparable workability of the alloys.

Some specimens were made from the profiles for tests of mechanical properties during tensioning at room temperature.

The tensile tests were performed on the flat specimens according to GOST 1497-84 made from the profiles in the hot-extruded state.

The mechanical test results are given in Table 4.

**Table 4**

| Alloy composition | Mechanical properties at 20°C | | |
|---|---|---|---|
| | Ultimate tensile strength, σ_{B}, MPa | Yield strength σ_{0.2}, MPa | Percentage elongation δ, % |
| 1 | 320 | 195 | 16.5 |
| 2 | 325 | 197 | 15.5 |
| 3 | 320 | 190 | 15.7 |
| A | 314 | 186 | 15.0 |

As the comparison of mechanical properties of the profiles given in Table 4 shows, the offered alloys ensure higher strength properties versus the prototype, whilst keeping percentage elongation and workability during extrusion. The most significant advantage of the alloy is higher strength, which will allow reducing wall thickness of products made of it and thereby increasing weight efficiency of structures made of it.

### Example 3

Slabs 120x400x1200 mm in size were cast with the semi-continuous casting method. Chemical composition of the slabs is given in Table 5. The studies were made on the first and second alloy compositions meeting the formula of Si ≤ Zr+2Sc, as well as on the third and fourth alloy compositions not meeting the ratio.

After cutting of the head and bottom parts, the slabs were homogenised in the three-stage mode. First stage at temperature of 370-380°C for 3 h. Second stage at temperature of 450-460°C for 6 h. Blanks 100x340x320 mm in size for rolling were cut from the slabs after homogenisation. Hot rolling of the flat blanks was performed at temperatures of 440-460°C to thickness of 6 mm. After that, their intermediate annealing was performed at temperature of 290-330°C followed by cold rolling to thickness of 1.0 mm. The rolled sheets were annealed at temperature of 280-320°C.

Some specimens were cut from the sheets for tests of mechanical properties during tensioning at room temperature, corrosion resistance, and workability with the Erikson extrusion method.

The tensile tests were performed on the flat specimens according to GOST 1497-84. The process tests with the Erikson sheet extrusion method were performed according to GOST 10510-80. The intercrystalline corrosion tests were performed on the specimens 10x20 mm in size according to GOST 9.021-74 in solution 1 for 24 h.

The mechanical, process, and corrosion test results are given in Table 6.

**Table 6**

| Alloy composition | Mechanical properties at 20°C | | | Dimple depth, Erikson extrusion, mm | Intercrystalline corrosion, mm |
|---|---|---|---|---|---|
| | Ultimate tensile strength, σ_{B}, MPa | Yield strength σ_{0.2}, MPa | Percentage elongation δ, % | | |
| 1 | 310 | 195 | 20.5 | 8.0 | No |
| 2 | 320 | 170 | 23.5 | 8.7 | No |
| 3 | 310 | 160 | 18.0 | 7.5 | No |
| 4 | 320 | 170 | 18.4 | 7.2 | No |
| A (sheet, annealing) | 255 | 110 | 18.0 | 7.8 | No |

As the comparison of mechanical properties of the profiles given in Table 5 shows, a failure to observe the ratio of Si ≤ Zr+2Sc results in deterioration of plastic properties, which is characterised by reduction of percentage elongation and decrease of dimple depth during the Erikson tests.

The scope of legal protection is solicited for the non-heat-treatable wrought aluminium-based alloy containing magnesium, manganese, scandium, zirconium, silicon, titanium. At that, the alloy additionally contains at least one element from the group of copper and zinc, as well as at least one element from the group of boron and carbon, with the following ratio of components, % wt:

| | |
|---|---|
| Magnesium | 3.0-5.2 |
| Manganese | 0.15-1.0 |
| Scandium | 0.010-0.045 |
| Zirconium | 0.03-0.14 |
| Silicon | 0.025-0.180 |
| Titanium | 0.01-0.05 |
| Copper and zinc (in total or separately) | 0.01-0.55 |
| Boron and carbon (in total or separately) | 0.0001-0.005 |
| Aluminium and inevitable impurities | Balance |

It is advisable that the alloy additionally contains yttrium in quantity of 0.005-0.02% wt, as well as that contents of scandium, zirconium, silicon meet the ratio of Si ≤ Zr + 2Sc in order to exclude precipitation of triple phases with silicon and scandium and/or zirconium. At that, silicon content is kept without formation of Mg₂Si crystallisation phase and the alloy is not doped with chromium and beryllium.

This alloy allows production of rolled semi-finished products using one-stage, two-stage, or three-stage annealing with at least one annealing stage implemented at temperatures above solvus to ensure the most efficient action of hardening elements in the material. At that, the process ensures high properties of the material in the recrystallised state, namely: ultimate tensile strength not less than 300 MPa, yield strength not less than 160 MPa, and percentage elongation not less than 20%.

This alloy also ensures its implementation in form of extruded semi-finished products, whilst ensuring high properties of the material, namely: ultimate strength not less than 320 MPa, yield strength not less than 190 MPa, and percentage elongation not less than 15.5%.

The alloy is also can be used for production with the cold deformation method from sheet semi-finished products. At that, the material has high properties in the recrystallised state, namely: ultimate tensile strength not less than 300 MPa, yield strength not less than 160 MPa, and percentage elongation not less than 20%.

## Claims

1. Non-heat-treatable wrought aluminium-based alloy, which contains magnesium, manganese, scandium, zirconium, silicon, titanium, additionally contains at least one element of the group including copper and zinc, and additionally contains at least one element of the group including boron and carbon, with the following ratio of components, % wt:
| | |
|---|---|
| Magnesium | 3.0-5.2 |
| Manganese | 0.15-1.0 |
| Scandium | 0.010-0.045 |
| Zirconium | 0.03-0.14 |
| Silicon | 0.025-0.180 |
| Titanium | 0.01-0.05 |
| Copper and zinc (in total or separately) | 0.01-0.55 |
| Boron and carbon (in total or separately) | 0.0001-0.005 |
| Aluminium and inevitable impurities | Balance |

2. The alloy described in Claim 1 **characterised in that** it additionally contains yttrium in quantity of 0.005-0.02% wt.

3. The alloy described in Claim 1, where contents of scandium, zirconium, silicon meet the ratio of Si ≤ Zr + 2Sc in order to exclude precipitation of triple phases with silicon and scandium and/or zirconium.

4. The alloy described in Claim 1, where silicon content is kept without formation of Mg₂Si crystallisation phase and the alloy is not doped with chromium and beryllium.

5. The alloy described in any one of Claims 1-4, which allows production of rolled semi-finished products using one-stage, two-stage, or three-stage annealing with at least one annealing stage implemented at temperatures above solvus to ensure the most efficient action of hardening elements in the material; at that, the process ensures high properties of the material in the recrystallised state, namely: ultimate tensile strength not less than 300 MPa, yield strength not less than 160 MPa, and percentage elongation not less than 20%.

6. The alloy described in any one of Claims 1-4 which ensures its implementation in form of extruded semi-finished products, whilst ensuring high properties of the material, namely: ultimate strength not less than 320 MPa, yield strength not less than 190 MPa, and percentage elongation not less than 15.5%.

7. Products produced with the cold deformation method from sheet semi-finished products made of the aluminium alloy described in any one of Claims 1-5; wherein the material has high properties in the recrystallised state, namely: ultimate tensile strength not less than 300 MPa, yield strength not less than 160 MPa, and percentage elongation not less than 20%.
